

## UNITED STATES PATENT OFFICE

2,450,886

## SEMICONDUCTOR

Charles Alexander Escoffery, East Orange, N. J., and Madeline Duane Merva, Bernice, Pa., assignors to Federal Telephone and Radio Corporation, New York, N. Y., a corporation of Delaware

No Drawing. Application November 26, 1944,  
Serial No. 564,408

1 Claim. (Cl. 175—366)

1

The present invention relates to semi-conductors and particularly to high voltage selenium rectifiers.

It is quite important for dry type rectifiers, such as selenium rectifiers, that the forward-resistance is as low as possible and the back-resistance high. The resistance in the direction of flow is dependent upon the resistance of the semi-conducting layer, governed to a certain extent by the resistance voltage drop, the trend of the current-voltage curve, of the back-resistance layer, and the transition resistance of the semi-conducting surface to the supply electrode. This transition resistance must be as low as possible and must be independent of voltage if the operation of the rectifier is to be satisfactory. The characteristic resistance curve of the blocking layer itself is dependent upon its chemical and physical composition, and the magnitude of the resistances in both direction of current flow is primarily determined by the conductivity of the selenium itself.

It has been recognized before that the conductivity of selenium can be materially increased by a thorough conversion into a crystalline form by annealing it at a temperature close to the melting point and that the conductivity of selenium can be further increased by the addition of materials, such as pulverized halogen salts of heavy metals, alkalies, carbon powder, or organic compounds. After conversion the additional materials either appear as undecomposed matters having certain conductivity embodied in the selenium, or they are mainly decomposed into oxides or selenides of good conductivity. These latter are conductive bodies and form dangerous shunting paths in the selenium and in the blocking layer itself.

In view of these unfavorable results it was suggested to add to selenium such material which avoids impurities in the selenium layer. Realizing the advantage of adding pure halogens to pure selenium, it was tried to add halogens in their pure form to the selenium. However, difficulties were encountered to achieve a thorough mixture of the halogens and the selenium and as a further step in the advancement of the art and in the desire to avoid the forming of dangerous shunting paths in the selenium, it has been suggested to admix selenium-chloride or selenium-bromide to the selenium and to achieve in this way a better mixture between the halogens and the selenium, the latter being then essentially devoid of conducting residues.

The admixture of selenium-chloride or sele-

2

nium-bromide brought about an increase in the forward-conductivity of the blocking layer, but at the same time a proportionate increase in the back-conductivity had to be accepted.

Although the later proposal appeared to be another step in the advancement of the art, it did not provide satisfaction in those cases in which it was essential to increase the forward-conductivity of the rectifier without increasing at the same time the reverse-conductivity.

It is, therefore, the main object of the present invention to add such material to the selenium which not only avoids the formation of conducting residues in the selenium, and also avoids the formation of compounds of selenium with the metallic impurities, but at the same time increases the forward-conductivity of the rectifier without changing its reverse-conductivity, that means a decrease in the relation of forward-resistance to back-resistance, and allows also higher voltage than achieved before. This main object is achieved by adding one substance of the group of  $ICl$ ,  $IBr$ ,  $ICl_3$ ,  $IBr_2$ .

It is a further object of the present invention to provide one substance of the above mentioned group in relation of 100 weight parts of selenium to from .001 up to .5 weight part of the mentioned substance.

It is still another object of the present invention to provide a method of producing a semiconductor for selenium rectifiers which comprises admixing selenium with one substance from the group of  $ICl$ ,  $IBr$ ,  $ICl_3$ ,  $IBr_2$  in the mentioned relation.

For the achievement of the best possible conductivity and the highest increase of the forward-conductivity of the semi-conducting layer an admixture of the mentioned substance of .005 to .1 to selenium has been proven of particular benefit advantage.

The novel construction of the present rectifier has the advantage of using less rectifying discs within the rectifier stack for a certain predetermined forward-conductivity, where until now a greater number of rectifying discs had to be used.

There are different ways available to provide a thorough mixture of the halogen compound with the selenium. One way is, in case it is solid, as  $IBr$  and  $ICl_3$ , to pulverize the halogen compound and mix it with the selenium powder, another is to put the halogen compound such as  $ICl$  and  $IBr_2$ , into a crucible, which compound is covered thereafter with selenium, using the capacity of the mentioned compound to harden at

a temperature slightly below ordinary room temperature and to change into fumes by heating up the crucible, thereby streaming through the selenium positioned above it and mixing thoroughly with it. Still another way of adding one substance of the mentioned group of halogen compounds is to dissolve the substance in an alcohol, such as methyl, ethyl, etc., which alcohol will escape upon heating and the mentioned substance will remain in the selenium.

While we have disclosed the principles of our invention in connection with several different embodiments, it will be understood that these embodiments are given by way of example only and not as limiting the scope of the invention as set forth in the objects and the appended claim.

What we claim is:

In a process for manufacturing selenium rec-

4  
tifier elements the improvement that comprises incorporating in the selenium layer a minor proportion of a single substance selected from the class consisting of iodine compounds of chlorine and iodine compounds of bromine.

CHARLES ALEXANDER ESCOFFERY.  
MADELINE DUANE MERVA.

#### REFERENCES CITED

- 10 The following references are of record in the file of this patent:

#### UNITED STATES PATENTS

| Number    | Name              | Date           |
|-----------|-------------------|----------------|
| 2,173,249 | Boer et al. ----- | Sept. 19, 1939 |
| 2,226,715 | Geisler -----     | Dec. 31, 1940  |
| 2,227,827 | Dubar -----       | Jan. 7, 1941   |
| 2,316,905 | Waibel -----      | Apr. 20, 1943  |